

March 15, 1932.

L. G. FIRTH

**1,849,367**

## INGOT

Original Filed Aug. 12, 1929



**INVENTOR**

Lewis Gerald Hirth  
by  
Bryant & Stratton,  
Parrish & Blaikie, Agents

## UNITED STATES PATENT OFFICE

LEWIS GERALD FIRTH, OF PITTSBURGH, PENNSYLVANIA, ASSIGNOR TO FIRTH-STERLING STEEL COMPANY, OF MCKEESPORT, PENNSYLVANIA, A CORPORATION OF PENNSYLVANIA

## INGOT

Original application filed August 12, 1929, Serial No. 385,255. Divided and this application filed August 16, 1930. Serial No. 475,721.

This invention relates to ingot molds having deep recesses in its molding surfaces for forming well defined severable flanges on an ingot cast in the mold, and to an ingot having a central body portion of relatively porous metal and well defined longitudinally severable flanges of relatively non-porous metal extending from the body portion.

Ingots of steel or other metals or alloys are now usually cast in molds having a substantially square cross-section. The ingot molds are sometimes provided with hot-tops through which the metal is poured into the mold, the hot-tops being used to keep the metal in liquid condition, thereby tending to decrease the amount of shrinks, pipes, and porosity of the cast ingot. Even with the use of hot-tops, however, the ingots are somewhat porous and for certain purposes it is necessary to scrap a large proportion of the ingot and use only that portion of the ingot which is substantially entirely free from porosity, segregation and shrinks. In making pistons for pneumatic rock-drills, valve seats and valves which are to be subjected to great pressures, or for airplane work, or other similar usages, it is necessary that the metal be substantially free from defects such as segregation, shrinks, or porous structure.

My invention is particularly adapted where it is necessary that the ingot be substantially free from the defects above mentioned. The usual process of casting ingots as practiced at the present time is to pour in such a way that the last portion to cool is at the top of the ingot and may be discarded. However, in any given cross section of an ingot at right angles to its longitudinal axis, the last portion to cool is the extreme center. It is probable that the central 5% to 15% of this cross section cools almost simultaneously, i. e., the solidification is progressive from the sides of the mold up to a certain point, at which point more or less simultaneous freezing takes place. It is this central 5% to 15% which contains the greater part of the segregated impurities and gases. This central portion also usually cools progressively from the bottom of the ingot to the top and it is customary to discard the upper portion or pipe end

which, generally speaking, is the last portion to cool. It is impracticable, however, under present practice to discard the whole of that central axis or core which extends from the bottom to the top of the ingot and which contains the steel last to cool in each horizontal plane.

In my invention, I not only discard the top portion of the ingot, according to common practice, but I also sever the ingot longitudinally and discard that portion in each horizontal plane which was the last to cool. It is in this respect that my invention differs radically from present day practice. The approximate amount of this last cooled portion to be removed according to my process is from 10% to 30% of the original weight of the ingot, this being taken mainly from the central portion of the casting. When a very high degree of perfection is required, as much as 50% of the original weight may be removed from the central portion. This can be regulated by cutting the ingot nearer or further from its central axis.

In my reference to "horizontal planes" and "longitudinal axis" I refer to ingots cast upright according to the usual practice, but my invention can also be applied when the ingot is cast with the longitudinal axis sloping or horizontal, and using either top or bottom pouring, or a combination of both.

In accordance with my invention, the ingot is cast in a mold having deep recesses formed therein which form flanges on the ingot extending outwardly from the body portion of the ingot. Any shrinks, pipes, or porous structure which may be present in the ingot are in the central portion thereof, and the flanges are free from such defects. The flanges are then separated from the relatively porous body portion and are worked by rolling or other shaping methods to form the desired articles.

This application is a division of my Patent No. 1,792,581, granted February 17, 1931.

Various shaped ingot molds are now employed to produce ingots which have a decreased tendency when rolled to form corner cracks and surface cracks. One type of such ingots has the cross sectional shape of a

55

60

65

70

75

80

85

90

95

100

dodecagon, and in one form of the dodecagon type, the ingot mold has four primary side walls and four outwardly arched corner walls, the primary side walls and corner walls being joined by inwardly bellied secondary corner walls. Such an ingot mold is described in Gathmann Patent, No. 1,719,543 and is designed to decrease corner and surface cracks when rolling large ingots.

10 The ingot mold of the present invention differs from that described in the above referred to Gathmann patent or from similar types by the fact that in the present invention the ingot mold is provided with deep recesses in its molding surfaces for forming well defined flanges which may be severed from the body portion of the ingot, and the severed flanges may thereafter be formed into the desired article. Any recesses formed 15 in the ingot mold according to the Gathmann patent above referred to are merely incidental to producing a contour of ingot such that corner cracks and surface cracks will be reduced when the ingot is rolled. The 20 recesses in the ingot mold are not of sufficient depth to provide well defined flanges which can be severed longitudinally from the body of the ingot and formed into the desired article.

25 30 In the accompanying drawings, which illustrate several present preferred embodiments of my invention;

Figure 1 is an elevation of an ingot mold;

Figure 2 is a section on the line II—II of 35 Figure 1; showing the ingot in the mold;

Figures 3 and 4 are sections similar to Figure 2, but showing ingots having four and five flanges, respectively;

Figure 5 is a section similar to Figures 2, 40 3 and 4, but showing another modification;

Figure 6 is a horizontal section of one of the flanges formed on the ingot, after the flange has been separated from the body portion of the ingot; and

45 Figure 7 is a perspective view of a rock-drill piston.

Referring more particularly to Figures 1 and 2 of the drawings, there is shown an ingot mold 2 which is generally triangular in 50 shape. The mold is formed of sections 3, 4 and 5, which are bolted together by bolts 6 and nuts 7. The mold provides deep recesses 8 extending radially from a central recess 9 which forms the body portion of the 55 ingot. The recesses 8 taper outwardly from the central portion of the mold, for a purpose hereinafter described.

In casting an ingot in the illustrated mold, the metal is poured in the usual manner, 60 preferably through a hot-top. The metal flows into the recesses 8 to form an ingot having a central body portion 10 and flanges 11 extending therefrom. Each of the flanges 11 has its three outer sides cooled by the mold. 65 The side of the flange 11, which is connected

to the central portion 10 of the ingot, remains hot for a longer time than the other sides of the flanges which contact with the mold sections. The cooling action of the ingot takes place first on the sides exposed 70 to the mold sections so that the flanges 11 are formed without shrinks, porous spots, or segregation. The only porous portion of the ingot is the central portion 10.

The flanges 11 are then separated along 75 the lines 15 from the central portion of the ingot which was the last portion to cool. After separation, the flanges, which are entirely solid, are rolled, forged, or otherwise shaped into the desired articles.

80 The ingot shown in Figure 3 is similar to the ingot of Figure 2, except that in Figure 3 the ingot has four flanges 11a instead of three. An ordinary mold 20 of substantially square cross section can be converted into a 85 mold embodying my invention by inserting filler blocks 21 in the corners of the mold in order to form a mold having recesses 8a which form flanges 11a on the body portion of the ingot, a body portion being that portion of 90 the ingot enclosed by the dotted lines 15a. When the mold shown in Figure 3 is used for casting the ingot, the flanges 11a are separated along the lines 15a from the central portion of the ingot.

95 In Figure 4 there is shown a mold having five recesses 8b, which form an ingot having five flanges 11b extending radially therefrom. My invention contemplates the formation of an ingot having any number of flanges 100 formed thereon.

105 In Figure 5 another form of ingot mold is shown. This mold has recesses 8c formed therein, which form the flanges 11c on the ingot. It also has recesses 25 provided in the mold which form flanges 26 on the ingot. When a mold of this shape is employed, the flanges 8c are separated from the remainder of the ingot along the lines 15c and only the two flanges 11c are worked to form the desired articles. The recesses 25 in the mold and the corresponding flanges 26 formed on the ingot are provided in order to cause the shrinks and segregations to take place as indicated at 27, and in order that the flanges 11c will be free from such defects.

110 In each of the embodiments, the flanges are separated by well defined recesses extending inwardly to points close to the body portion of the ingot. Thus, for example, in the embodiment shown in Figure 3, the flanges 11a are separated by well defined recesses 40a formed by the filler blocks 21. The recesses 40a extend close to the body portion of the ingot, which is that portion enclosed by the 115 dotted lines 15a.

120 The illustrated molds are made in sections which are bolted together, but, if desired, solid molds may be employed instead of split molds, and any number of recesses may be 125

provided in the molds to form a corresponding number of flanges on the ingots.

The recesses 8, 8a, 8b and 8c, preferably slope outwardly from the central portion of 5 the mold. In Figure 6 there is illustrated a flange 11 formed in the mold illustrated in Figure 2. As above stated, the flanges 11 are substantially free from porosity and segregation. However, there is a small portion 12 10 of the flange which is not quite as dense as the remaining portion of the flange. This is due to the fact that the portion 12 is the last to cool. In order to make the density of the billet rolled from the flange 11 absolutely 15 uniform, the flanges are cast having a slight taper outwardly from the central portion of the ingot. The inner portion 30 of the flange accordingly is subjected to greater work than the outer portion 31 when the flange is 20 rolled. The greater amount of work to which the portion 30 is subjected gives the rolled billet substantially uniform density throughout.

After rolling, forging, or otherwise shaping 25 the flange 11, it is formed into the desired article.

A piston 35 for a rock-drill is illustrated in Figure 7. Pistons made according to my invention are free from porosity, shrinks, and 30 other defects and are particularly adapted for the work which they have to perform. If a piston for a rock-drill is slightly porous, it is likely to crack under the strain imposed by the terrific impact of the piston against 35 the other parts of the rock-drill.

My invention is especially useful in the production of alloy steel articles which are expensive and in which it is desired to reduce to a minimum the portion of the ingot which 40 it is necessary to discard because of its porous character.

If desired, the ingot may be cast into molds which are rotated in order to force the metal from the central portion of the mold into 45 the recesses which form the flanges on the ingot.

I have illustrated and described several preferred forms of the invention. It is to be understood, however, that the invention 50 may be otherwise embodied within the scope of the following claims.

I claim:

1. An ingot having a body portion, and 55 at least three well defined severable flanges projecting outwardly beyond the body portion for a substantial distance, the flanges being separated by well defined recesses extending inwardly to points close to the body portion, the flanges being substantially free 60 from segregation, shrinks, and pipes, the volume of the metal in the flanges being greater than the volume of metal in the body portion.

2. An ingot having a body portion, and 65 at least three well defined severable flanges projecting outwardly beyond the body por-

tion for a substantial distance, the flanges being separated by well defined recesses extending inwardly to points close to the body portion, the flanges tapering outwardly from the body portion, the volume of the metal in 70 the flanges being greater than the volume of metal in the body portion.

3. An ingot having a body portion, and 75 well defined severable flanges projecting outwardly beyond the body portion for a substantial distance at angles of substantially 120°, the flanges being separated by well defined recesses extending inwardly to points close to the body portion, the volume of the metal in the flanges being greater than the volume of metal in the body portion.

4. An ingot having a body portion, and 80 well defined severable flanges projecting outwardly beyond the body portion for a substantial distance, the flanges being separated by well defined recesses extending inwardly to points close to the body portion, the cross section of the ingot in a plane transverse to its longitudinal axis being substantially cruciform, the flanges being substantially free 85 from segregation, shrinks and pipes, the volume of the metal in the flanges being greater than the volume of metal in the body portion.

In testimony whereof, I have hereunto set 90 my hand.

LEWIS GERALD FIRTH.

100

105

110

115

120

125

130